

Aug. 26, 1958

A. W. LEWING

2,849,000

TAMPONS AND THE LIKE

Filed June 8, 1953



INVENTOR  
ALBERT W. LEWING.

BY  
Curtis, Morris, Safford,  
ATTORNEYS

# United States Patent Office

2,849,000

Patented Aug. 26, 1958

1

2,849,000

## TAMPONS AND THE LIKE

Albert W. Lewing, Monson, Mass., assignor to Tampax, Incorporated, Palmer, Mass., a corporation of Delaware

Application June 8, 1953, Serial No. 360,071

11 Claims. (Cl. 128—285)

This invention relates to body fluid absorption device and more particularly to a compressed mass of treated absorbent fibers formed into a tampon or the like for insertion into a body cavity and adapted for increased absorption and retention of body fluid. This application is a continuation-in-part of my copending applications Serial Nos. 188,921 and 188,935, both filed October 7, 1950, both now replaced by continuation-in-part applications.

In the manufacture of body fluid absorption devices such as vaginal tampons, dental rolls, surgical pads, and the like, from, for example, a mass of absorbent cotton fibers, it is possible to increase the absorption capacity of the fibrous material by special treatment of the cotton, control of density of the cotton mass, etc. Such treatments, however, often fail to increase the capacity of the fibrous mass for retaining fluid absorbed against the intermittent squeezing such as that to which a vaginal tampon is subjected during use by the normal movement and activity of the wearer, or a dental roll by muscular movement of the cheek or pressure from the dentist while working. In fact, many treatments of absorbent cotton which improve its absorbency have by the same action facilitated the ease with which absorbed fluid can be expelled or squeezed out of the cotton.

According to this invention, it has been discovered that an improved absorption device of the character described can be produced using an unspun mass of absorbent cotton as the absorbing medium by treating the cotton fibers with retention agents as set forth herein, and that such treatment not only increases the absorbency of the cotton for body fluid, but also increases the amount of body fluid which a given amount of cotton fiber will retain against normal squeezing.

It is accordingly a principal object of this invention to provide an improved body fluid absorption device of the character described having improved capacity for absorbing and retaining fluid under normal conditions of use.

Another object of this invention is to provide an improved vaginal tampon of the character described including an unspun mass of treated absorbent fibers and having a greater capacity for retaining catamenial fluid against expulsion by squeezing than a similar tampon of untreated cotton.

A further object of this invention is to provide an absorption device of the character described for insertion into a body cavity and having a smaller bulk for a given body fluid absorption and retention capacity.

Still another object of this invention is to provide for the manufacture of fluid absorption devices of the character described to increase the capacities of such devices for fluid retention under normal conditions of use.

Still another object of this invention is to provide materials and methods for treating absorbent fibers to produce fluid absorption devices of the character described having such improved fluid retention capacities.

Other objects and advantages will be apparent from

2

the following description, the accompanying drawing and the appended claims.

In the drawing:

Fig. 1 is an isometric view of a vaginal tampon embodying this invention;

Fig. 2 is a view partly in axial section, partly in plan, of the tampon of Fig. 1; and

Fig. 3 is a graph showing a series of comparative clinical test results with vaginal tampons embodying this invention.

Referring to the drawing, Figs. 1 and 2 show, as illustrative of one embodiment of this invention, a vaginal tampon adapted to be inserted into the vagina. Tampons and the like which may be inserted into the vaginal cavity have been in common use for many years and have been increasingly recognized as a superior means for caring for the menstrual flow. A convenient and desirable absorbing medium from which such an insertable tampon may be made is a mass of unspun absorbent cotton. Such fibers are conveniently compressed into a more or less cylindrical mass of more or less rigid form and size for ready insertion into the cavity.

With such tampons of a size comfortable to the wearer, their value to the wearer depends upon the length of time during which they effectively absorb and hold all the menstrual flow.

According to this invention, a mass of absorbent fibers is treated with retention agents as set out below and such treatment greatly enhances the capacity of the mass not only to absorb more fluid but also to carry and retain more fluid against expulsion by squeezing forces. As a result, a satisfactory tampon of given size gives more effective service or one of smaller size capable of the same service can be produced according to this invention.

As illustrative of the results obtained with absorption devices embodying this invention, it has been found by clinical tests that such tampons of a conveniently small size, when worn for a prescribed period much longer than is permissible with existing tampons, are capable of absorbing and retaining all catamenial fluid and providing a high safety factor so that possibility of leakage, soiled clothing or other embarrassment is precluded.

Thus, it has been discovered and demonstrated as a result of clinical tests, that approximately six to eight

grams of catamenial fluid represents an average flow during four to five hours of the menstrual period and that twelve to fourteen grams represents an approximation of the heaviest menstrual flow normally encountered in that length of time. Since four to five hours appears to be the usual and convenient period for wearing a single tampon, such period has here been taken as standard for purposes of demonstrating and comparing the advantageous results of this invention. For these same purposes, the expression "percent protection" is used herein as meaning that percentage of the tampons clinically evaluated which were reported by the user as giving complete protection (i. e., no leakage or discoloration of clothing, etc.) during the reported use.

Such clinical evaluation with the three normally used sizes of tampons emphasizes the advantages of this invention:

(1) With the large size tampon of the highest quality sold commercially prior to this invention, the percent protection drops to 90% when the flow during the use of the tampon increases to six or eight grams, and percent protection drops to 20% when the flow increases above the twelve to fourteen gram range. A tampon of the same weight of the same cotton but embodying this invention, having been treated with glycerine as described hereinafter, gives 100% protection throughout the six to eight gram range, and the percent protection does not

drop even as low as 90% until the flow increases above the fourteen to sixteen gram range.

(2) The percent protection with the medium size untreated tampon of highest commercially available quality drops to 90% at the six to eight gram range and as low as 20% above the twelve to fourteen gram range. But identical tampons treated with glycerine so as to embody this invention provide 99% protection throughout the six to eight gram range, do not drop below 90% protection until above the ten to twelve gram range, and still offer 80% protection throughout the fourteen to sixteen gram range.

(3) The percent protection of untreated highest commercial quality tampons of the smallest size drops as low as about 80% even in the range six to eight grams of flow, and as low as about 45% in the eight to ten gram range. Identical tampons treated with glycerine to embody this invention provide 100% protection up to eight grams of flow and 80% protection up to ten grams of flow.

It should be noted that the clinical method necessarily used for test involves differences in personal activity and differences in flow, etc., such that about a difference of 2-3% in percent protection must be regarded as within the expected experimental error. However, when the percent protection drops below 95% it is serious and may not be disregarded.

Figure 3 is a graph showing such comparative clinical test results with identical tampons some of which are treated with glycerine, some with ethylene glycol, some with propylene glycol and some with polyethylene glycol, all according to the present invention. Each tampon was worn by a menstruating woman in the usual manner. Each was weighed before use and upon removal, and upon removal determination was made as to any evidence that menstrual fluid had escaped. The used tampons were grouped according to the weight of the fluid absorbed and the percentage of those in each group which had allowed no external evidence of menstrual flow was recorded, and plotted on Figure 3 as "percent protection."

Although the exact explanation of how or why the liquid retention capacities of tampons are so increased by treatment according to this invention is not now certainly known, useful hypothesis can be made. For example, it is thought that wetting agent action is not responsible for the advantages of this invention, since experiments with wetting agents have indicated that, although more fluid may be absorbed, the wetting agent tends to cause excess fluid to be more readily squeezed out of the tampon just as it is more readily absorbed, thereby reducing rather than increasing the retention capacity; whereas the protection effected by fluid retention, as shown by the above mentioned tests, are far beyond any improvement shown by laboratory tests on absorbency or capacity to take up and hold the test fluid dripped onto the tampon.

It is to be noted that the retention agents of this invention apparently become more strongly bonded to the cotton fibers themselves than can be explained by mere wetting or absorption and, although retained on the surface of the fibers, appear to produce a relatively low surface action on fluids absorbed by the mass of fibers. For example, untreated absorbent cotton will hold approximately 18 to 20 times its weight of water, but such water is easily squeezed out. On the other hand, cotton from the same batch when treated according to this invention will absorb approximately 10% more fluid than the untreated cotton, but the treated tampon will provide as much as 50% greater retention in a tampon, and protection to the wearer. It is noted, furthermore, that, although some satisfactory retention agents according to this invention may have certain wetting agent properties, all wetting agents do not produce satisfactory retention and, conversely, materials which do produce satisfactory results are not generally included

in the class of so-called wetting agents. What is wanted is something which will cause the fluid to spread over the fibers rapidly and yet hold it against draining or squeezing. It appears that something analogous to chemical bonding occurs and the presence of hydrophilic groups is believed to be significant, especially OH groups and especially with such groups at opposite ends of the molecule. Thus, it is evident that the polyhydric alcohols and their esters are most effective to improve retention of the absorbed fluid.

Representative concentrations and materials of the class of retention agents which have been found to produce satisfactory results according to this invention are:

|                         | Percent |
|-------------------------|---------|
| Glycerine               | 1-15    |
| Sorbitol                | .5-4    |
| Mannitol                | .5-4    |
| Ethylene glycol         | .5-2    |
| Propylene glycol        | .25-4   |
| 20 Butylene glycol      | .5      |
| Diethylene glycol       | .5-4    |
| Dipropylene glycol      | 1-4     |
| Triethylene glycol      | .5-2    |
| 25 Tetraethylene glycol | .5-2    |

Also fluid polyethylene glycols (e. g., those of approximately 200 to 400 molecular weight) have been found satisfactory. Such retention agents are all hydrophilic, water soluble polyhydric materials. Particularly with vaginal tampons and the like, the retention agents should also be substantially physiologically inert and without deleterious effect on benign organisms normally and desirably present in the body cavity in which the tampon is worn. The higher molecular weight, more or less solid or waxy polyethylene glycols (e. g., of approximately 1500 molecular weight) have been found to give good retention capacities to absorbent cotton in concentrations of from .5 to 2%, although the consistency of such materials has been found to introduce some difficulty into the carding operation of processing the absorbent cotton.

I have also found that wetting agents (e. g., Nacconal, a sulfonated aryl alkyl wetting agent) can be used to hasten absorption in combination with one of the retention agents, without impairing the retention action. The wetting agent improves the "wicking" action of the cotton, which takes care of cases of so-called "gushing" flow. Without this improved wicking action, a tampon would fail to give complete protection against such "gushing flow" although it would still have adequate capacity for further absorption of normal menstrual flow.

The above noted concentrations are on the air dry weight of the cotton (i. e., with about 5% moisture in the cotton). As illustrative of appropriate concentration ranges, it has been found that glycerine, for example, may advantageously be applied within the range of from .1% to about 15% as noted. In this range the absorbency and retention capacities of the cotton are significantly increased but to varying degrees. With glycerine concentrations substantially above this range, however, an impairment of dimensional stability of compressed tampons, and to some extent also, an actual diminution of absorbing capacity is noted. A final concentration on the completed tampon of approximately .25% to .75% of glycerine on the air dry weight of the cotton has been found most advantageous for commercial use. Although lower and higher concentrations of glycerine increase the absorbency capacity of the cotton, it has been noted that the range of the order of .5% (4-6% for practical operation) glycerine produces the greatest increase in retention capacity. Substantially higher concentrations provide an increase of retention capacity, although it has been found that the increase attributable to substantially higher concentrations of glycerine in many cases does not warrant the cost of the additional treating material. In concentrations above approximately 20%, the presence

of glycerine on the fibers is apparent to the touch, and this may render a tampon so treated unpleasant to handle or undesirable from a commercial standpoint. In this connection it should be noted that the amount of retention agents applied is only that which will treat the surfaces of the individual fibers; and distinction must be drawn between a tampon so treated with a retention agent and a tampon carrying so much of such agent that an appreciable portion of the interstices between fibers available for absorbing body fluid is occupied by the retention agent.

The retention agent is advantageously applied to unspun absorbent cotton fibers before they are cut and formed into a tampon. Satisfactory results have been obtained by adding the retention agent to the water in the final washing step in the process of manufacturing and preparing absorbent cotton bats to be used in manufacture of tampons.

Thus, a 10% glycerine in water wash solution may be applied to the cotton instead of the usual wash solution in the usual manner, e. g., by spraying the bat immediately ahead of the final squeeze rolls just prior to drying. It has been found that approximately 100 cc. of glycerine-water solution is retained after squeezing by approximately 100 grams of absorbent cotton in this process. In situations where the viscosity of the retention agent is sufficiently low to penetrate the mass of cotton fibers satisfactorily (e. g., where the process is carried out at sufficiently elevated temperatures and/or the fiber is wet at the time of application) undiluted agent may be directly applied to the cotton as by spraying. Also, other solvents than water (e. g., alcohol) may satisfactorily be used in the treating solution but water is preferred, since it obviates many problems of solvent elimination and recovery.

After the retention agent is applied, the fibers are dried to remove the solvent by any convenient means such as passing the cotton on a conveyor through a drying tunnel with circulation of warm air. Satisfactory results are obtained where the temperature at the wet end of the tunnel is approximately 240° F. and approximately 212° F. at the dry end, with the cotton passing through this range of temperatures in approximately one-half hour.

It should be noted that a substantial percentage of the agent originally applied to the cotton may be lost by evaporation along with the water during the drying procedure. It has been determined, for example, that cotton initially containing glycerine in concentrations of 0.5% to 10%, when dried at 240° F. for four hours may lose as much as 50 to 75% of this initially retained glycerine. Utilizing the half hour drying procedure described above, the cotton fibers may lose as much as 50% of the glycerine. It has been determined, however, that, when the remaining glycerine concentration is reduced to approximately .37%, it appears to be quite stably bound to the fibers and no further substantial loss of glycerine occurs even after heating many hours at 260° F. Such expected losses should be taken into consideration in determining the amount of glycerine applied, in order to achieve the desired concentration on the fibers of the finished tampons.

After the uncut and unformed bats of absorbent cotton fibers are completely processed and treated with the material as noted above, the bats may be cut into pads or tampons and, if desired, may be compressively formed into a desired size and shape by conventional means. By way of illustration, a convenient method of forming absorbent cotton fibers into a compressed, generally cylindrical tampon is indicated in the patents to Voss, No. 2,076,389, April 6, 1937, and McLaughlin No. 2,416,706, March 4, 1947. As shown by these patents, the loose cotton bats or tampon blanks are fed in between compression dies which impart thereto the desired cylindrical shape and degree of compression. They are thence ejected into cylindrical chambers where their compression

and shape are maintained while heat is applied to set the fibers thereof in their compressed form. In commercial practice tampons embodying this invention have been produced in three general size groups, e. g., containing approximately 3.1 grams, 2.3 grams and 1.4 grams of cotton.

It will also be understood that the treating material may satisfactorily be applied to the cotton at some stage in the processing thereof other than during the last washing step as described above. The conventional mill operations, e. g., carding, to which absorbent cotton is usually subjected after washing and drying have been found, because of the mechanical working involved, to distribute the retention agent throughout the cotton mass. The retention agent may be satisfactorily applied, however, at any convenient stage of the cotton processing when the fiber mass is sufficiently open or the individual fibers sufficiently exposed to obtain effective application and distribution. Any subsequent loss by evaporation or washing, however, should be taken into consideration.

I claim:

1. An improved vaginal tampon adapted for catamenial fluid absorption and retention under normal conditions of use within a vaginal cavity comprising as a fluid absorbing and retaining means a compressed mass of absorbent cotton fibers, said fibers carrying substantially uniformly distributed thereover a hydrophilic, nontoxic, polyhydric alcohol, retention agent.

2. An improved vaginal tampon adapted for catamenial fluid absorption and retention under normal conditions of use within a vaginal cavity comprising as a fluid absorbing and retaining means a compressed mass of absorbent cotton fibers, said fibers carrying substantially uniformly distributed thereover a fluid, nontoxic, hydrophilic, polyhydric alcohol retention agent selected from the class consisting of sorbitol, mannitol, glycerine, glycols and glycol polymers.

3. An improved vaginal tampon adapted for catamenial fluid absorption and retention under normal conditions of use within a vaginal cavity comprising as a fluid absorbing and retaining means a compressed mass of absorbent cotton fibers, said fibers carrying approximately 0.1% to 15% by weight of a retention agent selected from the class consisting of sorbitol, mannitol, glycerine, glycols, and glycol polymers.

4. A device for absorption and retention of body fluids comprising as a fluid absorbing and retaining means a compressed mass of absorbent fibers having the absorption and retention capacity thereof increased by impregnation with a fluid hydrophilic material selected from the class consisting of glycerine, glycols, glycol polymers, sorbitol, and mannitol, said materials being distributed over said fibers in an amount less than about 15% of the air dry weight of said fibers.

5. An improved vaginal tampon adapted for catamenial fluid absorption and retention under normal conditions of use within a vaginal cavity comprising as a fluid absorbing and retaining means a compressed mass of absorbent cotton fibers, said fibers carrying glycerine as a retention agent in an amount approximately 0.25% to 1% of the air dry weight of said cotton.

6. An improved vaginal tampon adapted for catamenial fluid absorption and retention under normal conditions of use within a vaginal cavity comprising as a fluid absorbing and retaining means a compressed mass of absorbent cotton fibers, said fibers carrying a fluid glycol retention agent in an amount approximately 0.25% to 1% of the air dry weight of said cotton.

7. An improved vaginal tampon adapted for catamenial fluid absorption and retention under normal conditions of use within a vaginal cavity comprising as a fluid absorbing and retaining means a compressed mass of absorbent cotton fibers, said fibers carrying glycerine as a retention agent in an amount approximately 0.1% to 15% of the air dry weight of said cotton.

8. An improved vaginal tampon adapted for catamenial fluid absorption and retention under normal conditions of use within a vaginal cavity comprising as a fluid absorbing and retaining means a compressed mass of absorbent cotton fibers, said fibers carrying glycerine as a retention agent in an amount approximately 0.4% to 0.6% of the air dry weight of said cotton.

9. An absorption device for insertion into a body cavity and adapted for body fluid absorption and retention under normal conditions of use comprising as a body fluid absorbing means a compressed mass of absorbent cotton fibers, said fibers carrying as a retention increasing agent ethylene glycol in an amount approximately 0.25% to 1% of the air dry weight of said cotton.

10. An absorption device for insertion into a body cavity and adapted for body fluid absorption and retention under normal conditions of use comprising as a body fluid absorbing means a compressed mass of absorbent cotton fibers, said fibers carrying as a retention increasing agent ethylene glycol in an amount approximately 0.4% to 0.6% of the air dry weight of said cotton.

5

11. An absorption device for insertion into a body cavity and adapted for body fluid absorption and retention under normal conditions of use comprising as a body fluid absorbing means a compressed mass of absorbent cotton fibers, said fibers carrying as a retention increasing agent a fluid polyethylene glycol in an amount approximately 0.25% to 1% of the air dry weight of said cotton.

10

References Cited in the file of this patent

UNITED STATES PATENTS

|           |               |               |
|-----------|---------------|---------------|
| 961,689   | Dorr -----    | June 14, 1910 |
| 2,095,377 | Breeze -----  | Oct. 12, 1937 |
| 2,229,061 | Eustis -----  | Jan. 21, 1941 |
| 2,340,311 | Donovan ----- | Feb. 1, 1944  |
| 2,602,042 | Abbott -----  | July 1, 1952  |

15

20

|         |                     |               |
|---------|---------------------|---------------|
| 112,192 | Germany -----       | June 6, 1900  |
| 537,113 | Great Britain ----- | June 10, 1941 |
| 550,638 | Great Britain ----- | Jan. 18, 1943 |

FOREIGN PATENTS